

Oct. 17, 1939.

J. C. MORRELL

2,176,353

MANUFACTURE OF AUTOMOTIVE FUEL

Filed July 30, 1936



Inventor:  
Jacque C. Morrell  
By: Lee J. Gary  
Attorney

## UNITED STATES PATENT OFFICE

2,176,353

## MANUFACTURE OF AUTOMOTIVE FUEL

Jacque C. Morrell, Chicago, Ill., assignor to Universal Oil Products Company, Chicago, Ill., a corporation of Delaware

Application July 30, 1936, Serial No. 93,372

2 Claims. (Cl. 196—49)

This invention relates more particularly to the manufacture of hydrocarbon fuels suitable for use in motors of the compression-ignition type.

More specifically the invention is concerned with a process for the manufacture of fuels suitable for use in Diesel and similar engines by an adaptation of a cracking process in which motor fuel suitable for use in spark ignition engines is concurrently produced.

10 The characteristics of fuels which are to be used in compression-ignition engines and those which are to be used in spark-ignition engines are generally opposite. As is well known, the spark ignition engines used on motor vehicles 15 require a fuel of considerable volatility and of slow burning characteristics so that there is no cracking of the fuel during combustion or development of peak pressures which cause the phenomenon known as "knocking". In fuel-injection engines of the Diesel type wherein the 20 heat of compression is relied upon to cause ignition at a definite point in the cycle of combustion, the most reliable fuels are those which have a tendency to crack and produce reactive molecules or radicals which readily ignite in the 25 presence of air under the compression ratios utilized in Diesel engines which are commonly of the order of from 10:1 to 20:1.

Up until recently, with the limited use of the 30 Diesel engine in automotive vehicles, little attention has been paid to increasing the yields of suitable Diesel fuel fractions from petroleum and efforts have been principally concentrated upon the manufacture of gasoline of high antiknock value by cracking and reforming operations and by the use of antiknock agents such as tetra ethyl lead. The requirements of a suitable fuel for light Diesel engines which may be used on trucks and to some extent on pleasure 35 vehicles are generally met by straight run gas oil or fuel distillate fractions boiling within the approximate range of 400-700° F. and it has been found that the higher the percentage of paraffins or readily "breakable" hydrocarbons in these fractions the more suitable they are for Diesel engine use. This property may be designated as paraffinicity, and it is commonly measured in terms of mixtures of the hydrocarbons cetane and alpha-methyl-naphthalene. 40 Prospective fuels are tested in a standard Diesel engine hook-up and the compression ratio found at which they ignite, and varying blends of the two chemical compounds mentioned are employed in comparison until one is found which ignites at the same compression ratio as the pro-

posed fuel, which is then given a cetane number rating corresponding to the percentage of this compound in the blend.

Ordinarily the cracking reaction, which has a tendency to produce unsaturated and cyclic hydrocarbons, does not produce Diesel fuel fractions of superior characteristics. However, by limiting the reactions of cracking to the primary reactions which do not extend to the formation of material amounts of cyclic hydrocarbons, Diesel fractions of suitable characteristics can be produced in economical quantities. It has been shown that the breaking down of a heavy oil into gasoline and gas may be preceded by the formation of intermediate fractions and the present 15 invention utilizes this fact for the production of Diesel fuels.

In one specific embodiment the present invention comprises cracking heavy petroleum fractions under conditions of time, temperature and pressure conducive to the formation of high yields of intermediate Diesel fuel fractions and separately cracking residual heavier fractions from this operation to produce gasoline of good antiknock value.

The present process thus consists of a series of cooperative steps in which both Diesel fuel and gasoline are produced by cracking, and in order to illustrate the general steps of the process the attached drawing has been provided, 30 which indicates diagrammatically in side elevation by the use of conventional figures an arrangement of apparatus in which the process may be conducted.

Referring to the drawing, charging oils are admitted by way of line 1 containing control valve 2 to a charging pump 3, which discharges by way of line 4 containing control valve 5 into and through a tubular heating element 6 disposed to receive heat from a furnace 7. The preferred 40 charging stocks are those which contain relatively low percentages of gas oil fractions and which have a paraffinic or mixed base character. The best stock is a paraffinic residue which contains very little material boiling below 500° F. 45 Naphthenic or asphaltic residue are not as suitable since they consist to a large extent of cyclic and poly-cyclic hydrocarbons which have high coke-forming tendencies and which tend to produce intermediate cracked distillates of a cyclic 50 character having relatively high antiknock characteristics which are not desirable in a Diesel fuel.

According to the present invention it is proposed to limit the reactions of decomposition as 55

far as practical to those of a primary character in the first stage of the process. Thus, relatively high temperatures of the order of 950 to 1100° F. and low time factors of the order of less than 5 seconds are preferably employed in the heating and reaction zones. The pressure factor is important in determining the capacity of equipment but is not necessarily controlling.

The heated products from heater 6 pass 10 through line 8 containing control valve 9 to a reaction chamber 10, which is proportioned, along with the capacity of the heating element, to give the proper time factor in connection with the feed rate employed.

15 The total products from the reaction chamber may be discharged through line 11 containing control valve 12 into a reduced pressure evaporator 13, which functions to separate vapors containing Diesel fuel fractions and lighter fractions 20 unavoidably produced from the heavier residual material. The vapor mixture passes through line 14 containing control valve 15 into a fractionator 16, which in turn serves to separate lighter overhead fractions and a Diesel fuel reflux. The 25 overhead vapors pass through line 17 containing control valve 18 and the condensable portions thereof are liquefied during passage through a condenser 19 and passed together with uncondensed gases through line 20 containing control 30 valve 21 to a distillate receiver 23 having the conventional gas release line 24 containing control valve 25 and a liquid draw line 26 containing control valve 27. The liquid produced at this point will generally be a good cracked gasoline which 35 can be blended with the corresponding product from the second stage of the process as desired.

The Diesel fuel fractions are removed from the bottom of fractionator 16 by way of line 28 containing control valve 29 and pass through a cooler 40 68 and thence through line 69 containing control valve 70 to a receiver 30, which also is provided with a gas release line 31 containing control valve 32 and a liquid line 33 containing control valve 34.

The hot residual products accumulating in 45 evaporator 13 are taken by way of line 35 containing control valve 36 to a pump 37 and discharged through line 38 containing control valve 39 into a heating element 40 arranged in a furnace setting 50 41. The conditions of cracking in this secondary system are preferably more severe than those employed in the primary system, particularly in regard to increased pressure and time factor, the former only being limited by the tendency of the residue to deposit coke in the heater tubes and 55 introduced hazards on account of local overheating. Temperatures of the order of from 850 to 950° F. are preferably employed at this point, and pressures as high as 500 pounds per square inch or higher may be used. Time factors are of the order of 10 to 40 seconds depending upon the character of the stock introduced and the temperature employed.

The products from heater 40 pass through line 60 42 containing control valve 43 into a reaction chamber 44, which is of a suitable capacity to permit the use of the preferred time factors and which may be insulated to conserve heat necessary for the completion of the cracking reactions.

70 The total products from chamber 44 are transferred by way of line 45 containing control valve 46 to a reduced pressure evaporator 47, which is ordinarily operated at pressures from approximately 50 to 100 pounds per square inch and 75 from which residues unsuitable for further con-

version are withdrawn through line 48 containing control valve 49 for use as fuel.

Vapors from evaporator 47 pass through line 50 containing control valve 51 to a second stage fractionator 52, which functions to separate the vapors into those comprising gasoline and fixed gases and heavier intermediate refluxes suitable for further conversion. The overhead passes through line 53 containing control valve 54 and through a condenser 55, in which the gasoline vapors are liquefied to pass with uncondensed gases through run-down line 56 containing control valve 57 to a receiver 58 having a gas release line 59 containing control valve 60 and a gasoline draw line 61 containing control valve 62.

10 The intermediate insufficiently converted refluxes pass through line 63 containing control valve 64 to a recycle pump 65, which discharges through line 66 containing control valve 67, back to line 38 and thence to the second stage 20 heating element 40 along with the primary residues from the first stage. A portion or all of the reflux may be withdrawn through line 66 controlled by valve 67 and passed through cooler 68, line 69 controlled by valve 70 into receiver 30 25 to augment the main supply of Diesel fuel oil product.

The following example is introduced to illustrate the type of results obtainable in practice by a process of the present character. It is 30 characteristic but is not introduced with the intent of limiting the scope of the invention correspondingly.

The charging stock to the process was a Mid-Continent topped crude which contained about 35 10% by volume of material boiling from 600-700° F., the remainder boiling above 700° F. This stock was given a light cracking at a temperature of 910° F. and a pressure of 200 lbs. per sq. in., the oil being exposed to these conditions 40 for a time of approximately 3 to 4 secs. As a result of this operation the following yields were obtained.

| Per cent<br>by weight         | 45 |
|-------------------------------|----|
| Fixed gas                     | 3  |
| 437° F. end point gasoline    | 10 |
| Intermediate distillate stock | 20 |
| Residuum                      | 67 |

The intermediate fraction in the above tabulation had a cetane number of approximately 45.

The residuum from the primary cracking step was then further cracked using a temperature of 935° F. and a pressure of 300 lbs. per sq. in., and 55 a time of approximately 30 secs. in the heating and cracking zones. The following tabulation indicates the yields of products by volume based on the primary residuum charged.

| Per cent                   | 60 |
|----------------------------|----|
| 405° F. end point gasoline | 50 |
| Cracked residuum           | 40 |
| Gas                        | 10 |

The blend of gasoline from the primary and secondary cracking steps had an octane number of 65 68-70 by the motor method, and the cracked residuum was low in suspended carbonaceous material so that it could be marketed directly as a Bunker fuel.

70 The nature of the present invention and its commercial value can be seen from the preceding specification and single example though neither section is intended to be unduly limiting upon its generally broad scope.

I claim as my invention:

1. A process for producing Diesel engine fuel and fuel for spark ignition engines from paraffinic and mixed base residues heavier than gas oil, which comprises, subjecting such residue to a temperature of from about 950 to 1100° F. for a cracking time of the order of less than five seconds, separating resultant vapors from unvaporized oil, fractionally condensing the vapors to form a condensate of hydrocarbons heavier than gasoline and removing this condensate from the process, subjecting said unvaporized oil to a temperature of from about 850 to 950° F. for a time period ranging from about 10 to 40 seconds to convert a substantial portion thereof into gasoline, fractionating the vapors formed by the last-named cracking treatment to condense fractions thereof heavier than gasoline, and finally condensing and collecting the fractionated vapors. 5
2. A process for producing Diesel engine fuel and fuel for spark ignition engines from paraffinic and mixed base residues heavier than gas oil, which comprises subjecting such residue to a temperature of from about 950 to 1100° F. for a cracking time of the order of less than five seconds, separating resultant vapors from unvaporized oil, fractionally condensing the vapors to form a condensate of hydrocarbons heavier than gasoline and removing this condensate from the process, subjecting said unvaporized oil to a temperature of from about 850 to 950° F. for a time period ranging from about 10 to 40 seconds to convert a substantial portion thereof into gasoline, fractionating the vapors formed by the last-named cracking treatment to condense fractions thereof heavier than gasoline, and finally condensing and collecting the fractionated vapors. 10
- 15
- 20

and mixed base residues heavier than gas oil, which comprises subjecting such residue to a temperature of from about 950 to 1100° F. for a cracking time of the order of less than 5 seconds, separating resultant vapors from unvaporized oil, fractionally condensing the vapors to form a condensate of hydrocarbons heavier than gasoline and removing this condensate from the process, subjecting said unvaporized oil to a temperature of from about 850 to 950° F. for a time period ranging from about 10 to 40 seconds to convert a substantial portion thereof into gasoline, fractionating the vapors formed by the last-named cracking treatment to condense fractions thereof heavier than gasoline, combining at least a portion of the resultant reflux condensate with the first-named condensate and recovering the resultant blend as the Diesel fuel product of the process, and finally condensing and collecting the fractionated vapors. 15

JACQUE C. MORRELL. 20